

## UNITED STATES PATENT OFFICE

2,511,938

PAD DYEING OF CELLULOSE DERIVATIVE  
FABRICS MADE FROM SIZED SPUN STAPLE  
FIBERS FOLLOWED BY DESIZINGWilfred T. Normand, Cumberland, Md., assignor  
to Celanese Corporation of America, a corpora-  
tion of DelawareNo Drawing. Application September 26, 1947,  
Serial No. 776,419

7 Claims. (Cl. 8—19)

1

This invention relates to the dyeing of fabric materials and relates more particularly to the dyeing of fabric materials made of or containing spun yarns of staple fibers having a basis of cellulose acetate or other organic derivative of cellulose material.

An object of this invention is the provision of an improved process for the dyeing of fabric materials made of or containing spun yarns of staple fibers having a basis of cellulose acetate or other organic derivative of cellulose material whereby said fabrics may be dyed in even, level shades free of overdyed surface fibers.

Other objects of this invention will appear from the following detailed description.

In weaving fabrics, both the warp and filling yarns are usually sized with a suitable sizing composition prior to the weaving operation in order to impart a measure of physical protection to the yarns. The size placed on the yarns renders them smooth and, therefore, highly resistant to the abrasive action of the moving shuttle supplying the filling yarn and to the mutually abrasive action of the yarns. When dyeing a woven fabric containing the weaving size, the fabric is first scoured to remove the size and then dyed employing a suitable dyebath and dyeing procedure to obtain the desired shade. The sequence of steps comprising scouring and dyeing is satisfactory for many types of fabrics woven of or containing yarns having a basis of cellulose acetate or other organic derivative of cellulose. However, it has been observed that when fabrics woven of or containing spun yarns of staple fibers having a basis of cellulose acetate or other organic derivative of cellulose material are first scoured and dyeing then effected by a mechanical impregnation method such as padding, the staple fiber ends which project from the surface of the fabrics are dyed a considerably deeper shade than the main body of the fabric. This results in a dyed fabric presenting an unevenly dyed appearance.

I have now found that fabrics made of or containing spun yarns of staple fibers of cellulose acetate or other organic derivative of cellulose material may be dyed rapidly in even, level shades by mechanical impregnation methods, such as pad-dyeing, and without any overdyeing of the surface fibers if said fabrics are dyed in the raw state, without prior scouring, and while still containing the size originally placed thereon to aid the weaving operation. The most advantageous results are obtained, in accordance with my novel process, if the dyebath employed for dyeing said raw, sized fabrics by mechanical impregnation methods comprises an aqueous alcohol solution of

2

the desired dyestuff containing a salt of thiocyanic acid which is a swelling agent for the cellulose acetate or other organic derivative of cellulose material. Surprisingly enough, the presence of the size on the fabric does not interfere with the dyeing of the fabric by said padding operation, as might normally be expected. Since the padding operation merely acts to thoroughly impregnate the fabric with the dyebath and does not exert any washing or scouring action on the sized fabric the fact that such even, level dyeings are obtained, despite the presence of the size, is quite unexpected. After dyeing is completed, the dyed fabric may be de-sized in a suitable scouring bath. The size employed may comprise a casein or gelatin base size, for example.

The lower aliphatic alcohols which are suitable for use in forming the solvent dyebaths which we employ for the pad-dyeing operation are those 20 alcohols which are solvents for the dyestuffs employed and which exert at least a swelling or softening action on the organic derivative of cellulose materials. While we prefer to employ ethyl alcohol in forming the dyebath, other alcohols such as methyl alcohol, propyl alcohol, isopropyl alcohol, n-butyl alcohol, secondary butyl alcohol, tertiary butyl alcohol, n-amyl alcohol, secondary amyl alcohol and tertiary amyl alcohol, or mixture of these alcohols may be used. The 30 amount of the alcohol used in the dye liquor will vary depending upon the alcohol or alcohols used. Optimum results are obtained when the lower aliphatic alcohol employed is ethyl alcohol and the latter comprises at least 60% by weight of the 35 dyebath.

As examples of swelling agents for the organic derivative of cellulose materials, there may be mentioned the salts of thiocyanic acid such as ammonium thiocyanate, sodium thiocyanate and 40 potassium thiocyanate, as well as other salts such as zinc thiocyanate. Optimum results are achieved employing sodium thiocyanate. The swelling agent is preferably present in amounts of from 1 to 3% on the weight of the dyebath.

45 Various dyestuffs for the cellulose acetate or organic derivative of cellulose materials may be employed in accordance with my novel process. The dyestuffs employed are preferably those dyes which are relatively insoluble in water and which 50 are usually applied to organic acid ester of cellulose materials in the form of aqueous dispersions. Mixtures of dyestuffs may also be employed.

The amount of dyestuff dissolved in the dyebath will, of course, vary with the final shade 55 desired in the material which is being dyed and may be from as low as 0.01% up to 5.0% based on the weight of the material to be dyed. Thus, as

a continuous process, the raw, sized fabric may be unwound from a roll, passed through a solution of the dyestuff, then between nipping rolls of a padding mangle which are adjusted to permit the desired amount of dye liquor to be retained in the fabric, and the fabric then subjected directly to washing or scouring whereby the size and any excess dyestuff removed. The duration of the immersion of the fabric in the dye liquor is relatively short and may be from 1 to 6 seconds. If desired, the fabric may be processed through the padding mangle at speeds ranging up to 60 yards per minute.

The staple fibers comprising the spun yarns in the fabrics dyed in accordance with my novel process may have a basis of cellulose acetate or other organic derivative of cellulose. Examples of other organic derivatives of cellulose are cellulose esters such as cellulose propionate, cellulose butyrate, cellulose acetate-propionate and cellulose acetatebutyrate, as well as cellulose ethers such as ethyl cellulose and benzyl cellulose.

In order further to illustrate my invention, but without being limited thereto, the following examples are given:

*Example I*

A warp of 150 denier, 40 filament cellulose acetate yarn and a 150 denier filling yarn spun of cellulose acetate staple fiber is sized with a size of the following composition applied on a slasher at 140° F.

|                    | Parts by weight |
|--------------------|-----------------|
| Casein             | 50              |
| Triethanolamine    | 10              |
| Triethyl phosphate | 3               |
| Water              | 1,000           |

The sized yarns are then woven in the usual manner into a heavy suiting fabric.

The woven fabric containing the weaving size is then padded through a dye solution of the following composition employing a suitable padding mangle:

|                                 | Parts by weight |
|---------------------------------|-----------------|
| Ethyl alcohol (95%)             | 60              |
| Water                           | 38              |
| Sodium thiocyanate              | 2               |
| 1:4-dimethylamino-anthraquinone | 1.5             |

The dyed fabric containing the weaving size is then set to a jig for two ends employing an aqueous scouring bath at 50° C. containing .06 gram per liter of sulfated lauryl alcohol and 3 grams per liter of a detergent mixture of sulfonated castor oil, xylene and water. The size is removed by this scouring bath. The scoured fabric is then dried and is found to be dyed in a level, even blue shade entirely free of overdyed surface fibers.

*Example II*

Cellulose acetate yarns of the deniers and construction described in Example I are sized on a slasher at 150° F. with a size of the following composition.

|                                    | Parts by weight |
|------------------------------------|-----------------|
| Gelatin                            | 50              |
| Sulfated fatty oil                 | 3.9             |
| Fatty oil                          | 3.9             |
| Soap                               | 1.7             |
| Water                              | 1,000           |
| Salt                               | 0.1             |
| Diethylene glycol mono-ethyl ether | 5               |
| Sodium ortho-phenyl phenate        | 0.5             |

The sized yarns are then woven into a heavy suiting fabric.

The woven fabric containing the weaving size is then padded through a dye solution of the following composition employing a suitable padding mangle:

|                                 | Parts by weight |
|---------------------------------|-----------------|
| Ethyl alcohol                   | 60              |
| Water                           | 38              |
| Sodium thiocyanate              | 2               |
| 1-hydroxy-4-amino-anthraquinone | 1.5             |

The dyed fabric containing the weaving size is then set to a jig for two ends and scoured as described in Example I to remove the size. The scoured fabric is dried and is found to be dyed in a level, even red shade free of overdyed surface fibers.

It is to be understood that the foregoing detailed description is given merely by way of illustration and that many variations may be made therein without departing from the spirit of my invention.

Having described my invention, what I desire to secure by Letters Patent is:

- 25 1. Process for the coloration of fabrics containing spun yarns of organic derivative of cellulose staple fibers, having thereon a proteinaceous size, in level, even shades free of overdyed surface fibers, which comprises padding said fabrics of said sized spun yarns with a solution of a dyestuff for the organic derivative of cellulose material in an aqueous medium comprising a lower aliphatic alcohol and an inorganic swelling agent for the organic derivative of cellulose material and then souring said dyed fabric to remove the size therefrom.
- 30 2. Process for the coloration of fabrics containing spun yarns of cellulose acetate staple fibers, having thereon a proteinaceous size, in level, even shades free of overdyed surface fibers, which comprises padding said fabrics of said sized spun yarns with a solution of a dyestuff for the cellulose acetate material in an aqueous medium comprising a lower aliphatic alcohol and an inorganic swelling agent for the cellulose acetate material and then scouring said dyed fabric to remove the size therefrom.
- 35 3. Process for the coloration of fabrics containing spun yarns of organic derivative of cellulose staple fibers, having thereon a proteinaceous size, in level, even shades free of overdyed surface fibers, which comprises padding said fabrics of said sized spun yarns with a solution of a dyestuff for the organic derivative of cellulose material in an aqueous medium comprising a lower aliphatic alcohol and a salt of thiocyanic acid which is a swelling agent for the organic derivative of cellulose material and then scouring said dyed fabric to remove the size therefrom.
- 40 4. Process for the coloration of fabrics containing spun yarns of cellulose acetate staple fibers, having thereon a proteinaceous size, in level, even shades free of overdyed surface fibers, which comprises padding said fabrics of said sized spun yarns with a solution of a dyestuff for the cellulose acetate material in an aqueous medium comprising a lower aliphatic alcohol and a salt of thiocyanic acid which is a swelling agent for the cellulose acetate material and then scouring said dyed fabric to remove the size therefrom.

- 45 5. Process for the coloration of fabrics containing spun yarns of organic derivative of cellulose staple fibers, having thereon a proteinaceous size, in level, even shades free of overdyed surface fibers, which comprises padding said fabrics of said sized spun yarns with a solution of a dyestuff for the organic derivative of cellulose material in an aqueous medium comprising a lower aliphatic alcohol and a salt of thiocyanic acid which is a swelling agent for the organic derivative of cellulose material and then scouring said dyed fabric to remove the size therefrom.
- 50 6. Process for the coloration of fabrics containing spun yarns of cellulose acetate staple fibers, having thereon a proteinaceous size, in level, even shades free of overdyed surface fibers, which comprises padding said fabrics of said sized spun yarns with a solution of a dyestuff for the cellulose acetate material in an aqueous medium comprising a lower aliphatic alcohol and a salt of thiocyanic acid which is a swelling agent for the cellulose acetate material and then scouring said dyed fabric to remove the size therefrom.
- 55 7. Process for the coloration of fabrics containing spun yarns of cellulose acetate staple fibers, having thereon a proteinaceous size, in level, even shades free of overdyed surface fibers, which comprises padding said fabrics of said sized spun yarns with a solution of a dyestuff for the organic derivative of cellulose material in an aqueous medium comprising a lower aliphatic alcohol and a salt of thiocyanic acid which is a swelling agent for the organic derivative of cellulose material and then scouring said dyed fabric to remove the size therefrom.
- 60 8. Process for the coloration of fabrics containing spun yarns of cellulose acetate staple fibers, having thereon a proteinaceous size, in level, even shades free of overdyed surface fibers, which comprises padding said fabrics of said sized spun yarns with a solution of a dyestuff for the cellulose acetate material in an aqueous medium comprising a lower aliphatic alcohol and a salt of thiocyanic acid which is a swelling agent for the cellulose acetate material and then scouring said dyed fabric to remove the size therefrom.

- 65 9. Process for the coloration of fabrics containing spun yarns of cellulose acetate staple fibers, having thereon a proteinaceous size, in level, even shades free of overdyed surface fibers, which comprises padding said fabrics of said sized spun yarns with a solution of a dyestuff for the cellulose acetate material in an aqueous medium comprising a lower aliphatic alcohol and a salt of thiocyanic acid which is a swelling agent for the cellulose acetate material and then scouring said dyed fabric to remove the size therefrom.
- 70 10. Process for the coloration of fabrics containing spun yarns of cellulose acetate staple fibers, having thereon a proteinaceous size, in level, even shades free of overdyed surface fibers, which comprises padding said fabrics of said sized spun yarns with a solution of a dyestuff for the organic derivative of cellulose material in an aqueous medium comprising a lower aliphatic alcohol and a salt of thiocyanic acid which is a swelling agent for the organic derivative of cellulose material and then scouring said dyed fabric to remove the size therefrom.

- 75 11. Process for the coloration of fabrics containing spun yarns of cellulose acetate staple fibers, having thereon a proteinaceous size, in level, even shades free from overdyed surface

fibers, which comprises padding said fabrics of said sized spun yarns with a solution of a dye-stuff for the cellulose acetate material in an aqueous medium comprising at least 60% by weight of ethyl alcohol and from 1 to 3% by weight of sodium thiocyanate and then scouring said dyed fabric to remove the size therefrom.

6. Process for the coloration of fabrics containing spun yarns of cellulose acetate staple fibers, having thereon a proteinaceous size, in 10 level, even shades free of overdyed surface fibers, which comprises padding said fabrics of said sized spun yarns with a solution of 1:4-dimethylamino-anthraquinone in an aqueous medium comprising at least 60% by weight of ethyl alcohol and from 1 to 3% by weight of sodium thiocyanate and then scouring said dyed fabric to remove the size therefrom.

7. Process for the coloration of fabrics containing spun yarns of cellulose acetate staple fibers, having thereon a proteinaceous size, in 15 level, even shades free of overdyed surface fibers, which comprises padding said fabrics of

6  
said sized spun yarns with a solution of 1-hydroxy-4-amino-anthraquinone in an aqueous medium comprising at least 60% by weight of ethyl alcohol and from 1 to 3% by weight of sodium thiocyanate and then scouring said dyed fabric to remove the size therefrom.

WILFRED T. NORMAND.

#### REFERENCES CITED

The following references are of record in the file of this patent:

#### UNITED STATES PATENTS

| Number    | Name      | Date          |
|-----------|-----------|---------------|
| 1,883,346 | Dreyfus   | Oct. 18, 1932 |
| 2,003,409 | Whitehead | June 4, 1935  |
| 2,274,751 | Sowter    | Mar. 3, 1942  |
| 2,428,835 | Croft     | Oct. 14, 1947 |

#### OTHER REFERENCES

20 Amer. Dye. Rep. for November 15, 1937, page 711.